

# UNITED STATES PATENT OFFICE.

ISADOR LADOFF, OF WILKINSBURG, PENNSYLVANIA, ASSIGNOR OF THIRTY ONE-HUNDREDTHS TO WALTER D. EDMONDS, OF BOONVILLE, NEW YORK.

## PROCESS OF PRODUCING ALLOYS.

1,221,873.

Specification of Letters Patent. Patented Apr. 10, 1917.

No Drawing.

Application filed October 12, 1915. Serial No. 55,418.

To all whom it may concern:

Be it known that I, ISADOR LADOFF, a citizen of the United States, residing at Wilkinsburg, in the county of Allegheny and State of Pennsylvania, have invented new and useful Improvements in Processes of Producing Alloys, of which the following is a specification.

My present invention relates to those processes of producing alloys by reduction of metallic oxids at temperatures sufficiently high to reduce such oxids without melting the resulting metals for which Letters Patent of the United States No. 1,040,699 were granted to me on October 8, 1912, and Letters Patent No. 1,042,694 on October 29, 1912.

The objects of my present invention comprise provision of expedients whereby as regards peculiarly refractory, or so to speak, more or less unmiscible, metals at the said temperatures may be caused to alloy as readily and perfectly as other metals. I have found that some few metals which are desirable in alloys for certain uses, such, for example, as uranium in alloy with ferro-metal for tool steels, prove, in operations conducted as per my said patents, practically unmiscible, or unalloyable with the ferro-metal, and that some other metals likewise desirable prove not as comprehensively miscible, or alloyable, as is, if only for economic reasons, desirable.

I have discovered, however, that if there be added to the charge during the operation a relatively unimportant, usually quite small, quantity of a compound, as for example the oxid of an element other than those intended to compose the alloy product, and the operation be otherwise conducted as per the specifications and certain of the claims of my said patents, as for example claims 1, 3, 4, 6, 8, 10, etc., of Patent No. 1,040,699, the oxids yield readily and to full extent desired their metallic constituents and in readily, homogeneously, and comprehensively alloying, or miscible, state, the resulting alloys being thus rendered more certain as to desired relative proportions of their constituents, and also caused to contain such percentages as desired of such hitherto especially refractory or unreadily miscible elements.

My invention is practised by first assembling, preferably in intimate mixture, the

oxids of the metals in proportions calculated to insure the respective percentages of the metals desired in the alloy. I incorporate, with this mixture, an auxiliary, to wit, another substance, the presence of which, during the operation, has, by my tests, been demonstrated to increase the percentage of properly alloyed difficultly miscible metal in the final product.

The charge is then subjected in presence of a reducing agent, to temperature below the melting points of said metals until the desired alloy has been produced.

My researches indicate that the additional or auxiliary substance incorporated in the charge as, and for, the purpose aforesaid, should preferably be an oxid, the reduction temperature of which is lower than that of the oxid of the more difficultly reducible and miscible of the to be alloyed metals, and also that it is preferable that the melting point of the element combined with oxygen in the oxid of the auxiliary substance should be lower than that of such difficulty miscible metal.

Said substance may be either a mineral, or usually preferably, a metallic compound. For example, I have found that arsenic tri-oxid ( $As_2O_3$ ) is thus very efficient as an added substance in the making, by my said process, of alloys of ferro-metals, or of copper, with such improving, but difficultly miscible metals as vanadium, or uranium; also that the same is true of antimony tri-oxid ( $Sb_2O_3$ ), and of the oxids of cobalt and nickel.

The proportion of the auxiliary substance added will, of course, depend upon the special requirements of each operation, and can, by usual tests, and experimentation, be readily determined by those skilled in the metallurgical art. The amount required is, for example, determinable by comparison of the quantity of the oxid of the relatively unmiscible metal used, with the percentage of such metal in the alloy, and the percentage of the auxiliary substance employed. The proportion required is, of course, as little more and as little less as possible to insure incorporation in the alloy of the full desired amount of the particular metal, or metals, which require to be thus assisted.

It will be apparent that the amount of the auxiliary substance to be added will, in some cases, be quite small. For example, in

the production of what are known as "tool steel alloys," *i. e.*, those in which such metals as vanadium or uranium are alloyed with the steel, the percentage of the oxids of such metals, in the charge, and of such metals in the alloy, is usually small compared to that of the ferro-metals, and consequently a correspondingly small addition of the auxiliary substance is required, say in many such cases 5 not to exceed five per centum of the charge. The residuum, if any, in the alloy of such small additions may usually be treated as negligible, or even as useful, as when oxids of metals are employed; but, in other cases, 10 the auxiliary may be, if desired, eliminated from the alloy by well known procedures, such, for example, as by, after its production by my method, raising the temperature of the alloy sufficiently to insure elimination 15 of therein remaining small quantities of arsenic.

Having now described my invention, what I claim as new and desire to secure by Letters Patent is the following, viz: 20

25 1. The method of producing an alloy which comprises mixing the oxids of its constituent metals, incorporating with the mixture a compound the reducing temperature of which is lower than that of one of said oxids, and subjecting the charge, in a reduc-

ing atmosphere, to temperature below the melting points of said metals but sufficiently high to inaugurate, and maintaining such temperature sufficiently long to insure, reduction of said oxids. 35

2. The method of producing an alloy which comprises mixing the oxids of its constituent metals, incorporating with the mixture another oxygen compound the reducing temperature of which is lower than that of one of said oxids, and subjecting the charge, in a reducing atmosphere, to temperature below the melting points of said metals but sufficiently high to inaugurate, and maintaining such temperature sufficiently long to insure, reduction of said oxids. 40

3. The method of producing an alloy which comprises mixing the oxids of its constituent metals, incorporating with the mixture an oxygen compound of arsenic, and subjecting the charge, in a reducing atmosphere, to temperature below the melting points of said metals but sufficiently high to inaugurate, and maintaining such temperature sufficiently long to insure, reduction of 45 said oxids. 50

ISADOR LADOFF.

Witnesses:

W. M. E. HAGUE,  
WEINMAN CRATTY.